# EUROPEAN PATENT SPECIFICATION

(11) **EP 0 540 297 B1**
(45) Date of publication and mention of the grant of the patent: **20.11.1996**
(21) Application number: 92309836.2
(22) Date of filing: 27.10.1992
(51) Int. Cl.: C10L 1/30

(54) **Unleaded aviation gasoline**
Bleifreies Flugbenzin
Essence non-plombée pour avion

(30) Priority: 28.10.1991 US 783210
(43) Date of publication of application: 05.05.1993
(73) Proprietor: ETHYL PETROLEUM ADDITIVES, INC., Richmond, Virginia 23219-4304 (US)
(72) Inventor: Henderson, Douglas Harold, Glen Allen, Virginia 23060 (US)
(74) Representative: Woods, Geoffrey Corlett

(56) References cited:
- EP-A- 0 466 511
- GB-A- 2 186 287
- KIRK-OTHMER 'ENCYCLOPEDIA OF CHEMICAL TECHNOLOGY EDITION 3,VOLUME 3' , JOHN WILEY AND SONS , NEW YORK
- NELSON 'PETROLEUM REFINERY ENGINEERING EDITION 4' , MC GRAW HILL , NEW YORK

## Description

This invention relates to unleaded aviation gasoline compositions which satisfy the specification requirements of ASTM Specification D910-90.

The specifications imposed upon aviation gasolines are necessarily extremely rigorous, since the consequences could be disastrous if an aviation gasoline does not perform properly in a spark-ignition aviation engine.

While leaded aviation gasolines have performed wonderfully well in actual service for many years, many misguided persons have clamored for elimination of lead from gasoline. If their efforts succeed, the refining industry will be faced with the problem of trying to provide unleaded aviation gasoline that performs as well as leaded aviation gasoline and that does not exceed the economic constraints of the marketplace.

This invention is deemed to overcome the above problem most expeditiously.

In accordance with this invention, there is provided an unleaded aviation gasoline composition which comprises a blend of hydrocarbons and at least one cyclopentadienyl manganese tricarbonyl compound dissolved therein in an amount such that said gasoline composition has a minimum knock value lean rating octane number of 100 as determined by ASTM Test Method D2700 and wherein Motor Method octane ratings are converted to aviation ratings in the manner described in ASTM Specification D910-90, said composition being further characterized by having: a) a distillation temperature as determined by ASTM Test Method D86 of 10% evaporated, 75°C (167°F) maximum temperature; 40% evaporated, 75°C (167°F) maximum temperature; 90% evaporated, 135°C (275°F) maximum temperature; and a final boiling point of 170°C (338°F) maximum temperature; the sum of the 10 and 50% evaporated temperatures being 152.8°C (307°F) minimum; the distillation recovery being 97% minimum; the distillation residue being 1.5% maximum; and the distillation loss being 1.5% maximum; b) a heat of combustion as determined by ASTM Test Method D1405 and as calculated from Table 1 thereof of 4.354x10⁷ J/kg (18,720 btu per pound) minimum, or a heat of combustion as determined by ASTM Test Method D2382 of 4.350x10⁷ J/kg (18,700 btu per pound) minimum, the latter method controlling in case of a discrepancy therebetween; c) a vapor pressure as determined by ASTM Test Method D323 or D2551 of 3866.89 kg/m² (5.5 psi) minimum and 4921.49 kg/m² (7.0 psi) maximum; d) a copper strip corrosion as determined by ASTM Test Method D130 of number 1, maximum; e) a potential gum (5-hour aging gum) as determined by ASTM Test Method D873 of 6 mg per 100 mL maximum, or a potential gum (16-hour aging gum as determined by ASTM Test Method D873) of 10 mg per 100 mL; f) a sulfur content as determined by ASTM Test Method D1266 or D2622 of 0.05% by weight maximum; g) a freezing point as determined by ASTM Test Method D2386 of - 22.2°C (72°F) maximum; and h) a water reaction as determined by ASTM Test Method D1094 wherein the volume change, if any, does not exceed ± 2 mL.

Preferred gasoline compositions are those in which the gasoline composition additionally has a minimum performance number reported to the nearest whole number and as determined by ASTM Test Method D909 of 130. In this connection, a minimum performance number of 130 is equivalent to a knock value determined using isooctane plus 1.28 milliliters of tetraethyllead per 3.79 Litres (per gallon).

Another embodiment of this invention provides the method of operating a four stroke cycle, reciprocating piston aircraft engine which comprises providing or using as the fuel for said engine a gasoline composition of this invention.

Cyclopentadienyl manganese tricarbonyl compounds which can be used in the practice of this invention include cyclopentadienyl manganese tricarbonyl, methylcyclopentadienyl manganese tricarbonyl, dimethylcyclopentadienyl manganese tricarbonyl, trimethylcyclopentadienyl manganese tricarbonyl, tetramethylcyclopentadienyl manganese tricarbonyl, pentamethylcyclopentadienyl manganese tricarbonyl, ethylcyclopentadienyl manganese tricarbonyl, diethylcyclopentadienyl manganese tricarbonyl, propylcyclopentadienyl manganese tricarbonyl, isopropylcyclopentadienyl manganese tricarbonyl, tert-butylcyclopentadienyl manganese tricarbonyl, octylcyclopentadienyl manganese tricarbonyl, dodecylcyclopentadienyl manganese tricarbonyl, ethylmethylcyclopentadienyl manganese tricarbonyl, and indenyl manganese tricarbonyl, including mixtures of two or more such compounds. Preferred are the cyclopentadienyl manganese tricarbonyls which are liquid at room temperature such as methylcyclopentadienyl manganese tricarbonyl, ethylcyclopentadienyl manganese tricarbonyl, liquid mixtures of cyclopentadienyl manganese tricarbonyl and methylcyclopentadienyl manganese tricarbonyl, and mixtures of methylcyclopentadienyl manganese tricarbonyl and ethylcyclopentadienyl manganese tricarbonyl. Preparation of such compounds is described in the literature, for example, U.S. 2,818,417.

In another preferred embodiment the unleaded gasoline composition additionally contains at least one antioxidant in an amount not in excess of 3.8 kg per 159 m³ (8.4 pounds per 1000 barrels), said antioxidant being selected from the group N,N'-diisopropyl-p-phenylenediamine, N,N'-di-sec-butyl-p-phenylenediamine, 2,4-dimethyl-6-tert-butylphenol, 2,6-di-tert-butyl-4-methylphenol, 2,6-di-tert-butylphenol, a mixture of 75% minimum 2,6-di-tert-butylphenol plus 25% maximum di- and tri-tert-butylphenol; and a mixture of 75% minimum di- and triisopropyl phenols plus 25% maximum di- and tri-tert-butylphenol. Most preferably the amount of such antioxidant does not exceed 1.9 kg per 159 m³ (4.2 pounds per 1000 barrels).

It is to be understood that the fuels of this invention are unleaded in the sense that a lead-containing antiknock agent is not deliberately added to the gasoline. Trace amounts of lead due to contamination of equipment or like circumstances are permissible and are not to be deemed excluded from the practice of this invention.

The base fuels used in the foregoing compositions can be blends of refined hydrocarbon derived from crude petroleum, natural gasoline, or blends thereof with synthetic hydrocarbons or aromatic hydrocarbons, or both. Blending components, if approved for use in aviation gasolines, such as oxygenated ingredients, can be included. Rarely, if ever, will the content of aromatic hydrocarbons in the gasoline exceed levels above 25%. As noted above, the overall composition must satisfy the requirements a) through h) inclusive as set forth above.

Other components which can be employed, and under certain circumstances are preferably employed, include dyes which do not contribute to excessive induction system deposits. Typical dyes which can be employed are 1,4-dialkylaminanthraquinone, p-diethylaminoazobenzene (Color Index No. 11020) or Color Index Solvent Yellow No. 107, methyl derivatives of azobenzene-4-azo-2-naphthol (methyl derivatives of Color Index No. 26105), alkyl derivatives of azobenzene-4-azo-2-naphthol, or equivalent materials. The amounts used should, wherever possible, conform to the limits specified in ASTM Specification D910-90.

Fuel system icing inhibitors may also be included in the fuels of this invention. Preferred are ethylene glycol monomethyl ether and isopropyl alcohol, although materials giving equivalent performance may be considered acceptable for use. Amounts used should, wherever possible, conform to the limits referred to in ASTM Specification D910-90.

The concentration of the cyclopentadienyl manganese tricarbonyl compound used in the unleaded aviation gasoline base stock satisfying the above criteria will vary to some extent depending upon the identity and properties of the base fuel and the octane quality desired in the finished fuel. Ordinarily amounts equivalent to 0.01-0.5 gram of manganese per gallon of fuel are sufficient, although higher amounts can be used whenever deemed necessary or appropriate, provided that the resultant fuel composition satisfies the requirements of a) through h) above. Preferably the fuel will contain up to 0.25 gram of manganese per 3.79 Litres (per gallon) as one or more cyclopentadienyl manganese tricarbonyl compounds.

There are good and sufficient reasons why the gasoline composition is to comply with the requirements set forth above as a) through h). The rationale behind these requirements as set forth in ASTM Specification D910-90, paragraphs X1.1.1, X1.1.3 and X1.2.1.

In accordance with other preferred embodiments this invention further provides a method of operating a four stroke cycle, reciprocating piston aircraft engine which comprises providing and/or using as the fuel for said engine a gasoline composition of this invention, and providing and/or using as the lubricating oil for said engine a lubricating oil composition satisfying the chemical and physical property requirements set forth below;

The chemical and physical property requirements of the lubricating oil used in the foregoing preferred aircraft engine embodiment are as follows:
1) Viscosity, m²/S (cSt), per ASTM D 445:

| SAE Grade | Minimum at 100°C | Less than at 100°C |
|---|---|---|
| 30 | 9.3x10⁻⁶ (9.3) | 12.5x10⁻⁶ (12.5) |
| 40 | 12.5x10⁻⁶ (12.5) | 16.3x10⁻⁶ (16.3) |
| 50 | 16.3x10⁻⁶ (16.3) | 21.9x10⁻⁶ (21.9) |
| 60 | 21.9x10⁻⁶ (21.9) | 26.1x10⁻⁶ (26.1) |

2) Multigrade oil shall meet the viscosity requirements and the Low Temperature Viscosity Cold Crank Simulation requirements of SAE Test Method J300 for the designated grade.
3) Viscosity Index, minimum per ASTM D 2270: 100 for SAE grades 30, 40 and Multigrade; 95 for SAE grades 50 and 60.
4) Flash Point, °C, minimum per ASTM D 92: 220 for SAE grades 30 and Multigrade; 225 for SAE grade 40; and 243 for SAE grades 50 and 60.
5) Pour Point, °C, maximum per ASTM D 97: -24 for SAE grade 30; -22 for SAE grade 40; and -18 for SAE grades 50 and 60.
6) Viscosity, High Temperature, High Shear at 150°C, Pas (cP) minimum per ASTM D 4683, D 4741, D 4624: 3.3x10⁻³ Pas (3.3) for all viscosity grades.
7) Total Acid Number, mg KOH/g, maximum (titrated to a pH 11 end point) per ASTM D 664: 1.0 for all viscosity grades.
8) Ash Content, Mass %, maximum per ASTM D 482: 0.006 for all viscosity grades.
9) Trace Sediment, mL/100 mL Oil, maximum per ASTM D 2273: 0.005 for all viscosity grades.
10) Copper Strip Corrosion, maximum rating per ASTM D 130: 1 after 3 hours @ 100°C for all viscosity grades; and 3 after 3 hours @ 204°C for all viscosity grades.
11) Foaming Tendency/Stability per ASTM D 892: Aerated Volume, mL, maximum for all viscosity grades per Sequences I, II and III: 50; Volume after 10 minutes, mL, maximum for all viscosity grades per Sequences 1, II, and III: 0.
12) Compatibility with other oils per FTM 791 Method 3403: All viscosity grades shall pass.
13) Elastomer Compatibility, % swelling, acceptable range for all viscosity grades after 72 hours per FTM 791 Method 3604 (except conducted with the specific materials and temperatures herein listed):

| Material | Test Temperature | Acceptable Limits |
|---|---|---|
| AMS-3217/1 | 70°C (158°F) | - 5 to + 5 |
| AMS-3217/4 | 150°C (302°F) | - 5 to + 5 |
| AMS-3217/5 | 150°C (302°F) | - 5 to + 5 |
| US Navy Silicone Rubber | 121°C (250°F) | 0 to + 20 |

14) Trace Metal Content, ppm, maximum for all viscosity grades, per test method of Paragraph 4.5.2 of MIL-L-22851D (1 December 1990) or equivalent: Iron, 5; Silver, 3; Aluminum, 7; Chromium, 5; Copper, 3; Magnesium, 3; Nickel, 3; Lead, 5; Silicon, 25; Tin, 10; Titanium, 2; Molybdenum, 4.

The most preferred lubricating oils will not only meet the above requirements 1) through 14) but in addition, will meet the following L-38 Engine Test Requirements:
15) Total Bearing Weight Loss, mg, maximum per ASTM STP 509A, Part IV for all viscosity grades: 500.
16) Used Oil Viscosity, Stripped, maximum % Change @ 40°C per ASTM D 445 for all single viscosity grades: -15 to + 10.
17) Used Oil Viscosity at 100°C of Multi-grade Oil per SAE J300 shall remain in SAE J300 grade.
18) Used Oil Total Acid Number, maximum change for all viscosity grades per ASTM D 664 (titrated to a pH 11 end point): 2.0.

## Claims

1. An unleaded aviation gasoline composition which comprises a blend of hydrocarbons and at least one cyclopentadienyl manganese tricarbonyl compound dissolved therein in an amount such that said gasoline composition has a minimum knock value lean rating octane number of 100 as determined by ASTM Test Method D2700 and wherein Motor Method octane ratings are converted to aviation ratings in the manner described in ASTM Specification D910-90, said composition being further characterized by having:
a) a distillation temperature as determined by ASTM Test Method D86 of 10% evaporated, 75°C (167°F) maximum temperature; 40% evaporated, 75°C (167°F) maximum temperature; 90% evaporated, 135°C (275°F) maximum temperature; and a final boiling point of 170°C (338°F) maximum temperature; the sum of the 10 and 50% evaporated temperatures being 152.8°C (307°F) minimum; the distillation recovery being 97% minimum; the distillation residue being 1.5% maximum; and the distillation loss being 1.5% maximum;
b) a heat of combustion as determined by ASTM Test Method D1405 and as calculated from Table 1 thereof of 4.354x10⁷ J/kg (18.720 btu per pound) minimum, or a heat of combustion as determined by ASTM Test Method D2382 of 4.350x10⁷ J/kg (18,700 btu per pound) minimum, the latter method controlling in case of a discrepancy therebetween;
c) a vapor pressure as determined by ASTM Test Method D323 or D2551 of 3866.89 kg/m² (5.5 psi) minimum and 4921.49 kg/m² (7.0 psi) maximum;
d) a copper strip corrosion as determined by ASTM Test Method D130 of number 1, maximum;
e) a potential gum (5-hour aging gum) as determined by ASTM Test Method D873 of 6 mg per 100 mL maximum, or a potential gum (16-hour aging gum as determined by ASTM Test Method D873) of 10 mg per 100 mL;
f) a sulfur content as determined by ASTM Test Method D1266 or D2622 of 0.05% by weight maximum;
g) a freezing point as determined by ASTM Test Method D2386 of -57.8°C (-72°F) maximum; and
h) a water reaction as determined by ASTM Test Method D1094 wherein the volume change, if any, does not exceed ± 2 mL.

2. A composition as claimed in Claim 1 wherein said gasoline composition has a minimum knock value lean rating octane number of 100 as determined by ASTM Test Method D2700 and a minimum performance number reported to the nearest whole number and as determined by ASTM Test Method D909 of 130.

3. A composition as claimed in Claim 1 wherein said cyclopentadienyl manganese tricarbonyl compound consists essentially of methylcyclopentadienyl manganese tricarbonyl.

4. The method of operating a four stroke cycle, reciprocating piston aircraft engine which comprises A) providing or using as the fuel for said engine an unleaded aviation gasoline composition which comprises a blend of hydrocarbons and at least one cyclopentadienyl manganese tricarbonyl compound dissolved therein in an amount such that said gasoline composition has a minimum knock value lean rating octane number of 100 as determined by ASTM Test Method D2700 and wherein Motor Method octane ratings are converted to aviation ratings in the manner described in ASTM Specification D910-90, said composition being further characterized by having:
a) a distillation temperature as determined by ASTM Test Method D86 of 10% evaporated, 75°C (167°F) maximum temperature; 40% evaporated, 75°C (167°F) maximum temperature; 90% evaporated, 135°C (275°F) maximum temperature; and a final boiling point of 170°C (338°F) maximum temperature; the sum of the 10 and 50% evaporated temperatures being 152.8°C (307°F) minimum; the distillation recovery being 97% minimum; the distillation residue being 1.5% maximum; and the distillation loss being 1.5% maximum;
b) a heat of combustion as determined by ASTM Test Method D1405 and as calculated from Table 1 thereof of 4.354x10⁷ J/kg (18,720 btu per pound) minimum, or a heat of combustion as determined by ASTM Test Method D2382 of 4.350x10⁷ J/kg (18,700 btu per pound) minimum, the latter method controlling in case of a discrepancy therebetween;
c) a vapor pressure as determined by ASTM Test Method D323 or D2551 of 3866.89 kg/m² (5.5 psi) minimum and 4921.49 kg/m² (7.0 psi) maximum;
d) a copper strip corrosion as determined by ASTM Test Method D130 of number 1, maximum;
e) a potential gum (5-hour aging gum) as determined by ASTM Test Method D873 of 6 mg per 100 mL maximum, or a potential gum (16-hour aging gum as determined by ASTM Test Method D873) of 10 mg per 100 mL;
f) a sulfur content as determined by ASTM Test Method D1266 or D2622 of 0.05% by weight maximum;
g) a freezing point as determined by ASTM Test Method D2386 of -57.8°C (-72°F) maximum; and
h) a water reaction as determined by ASTM Test Method D1094 wherein the volume change, if any, does not exceed ± 2 mL.

5. A method as claimed in Claim 4 wherein said gasoline composition has a minimum knock value lean rating octane number of 100 as determined by ASTM Test Method D2700 and a minimum performance number reported to the nearest whole number and as determined by ASTM Test Method D909 of 130.

6. A method as claimed in Claim 4 wherein said cyclopentadienyl manganese tricarbonyl compound consists essentially of methylcyclopentadienyl manganese tricarbonyl.

7. The method of operating a four stroke cycle, reciprocating piston aircraft engine according to claim 4 which additionally comprises: providing and/or using as the lubricating oil for said engine a lubricating oil composition satisfying the following chemical and physical property requirements:
1) Viscosity, m²/S (cSt) per ASTM D 445:
| SAE Grade | Minimum at 100°C | Less than at 100°C |
|---|---|---|
| 30 | 9.3x10⁻⁶ (9.3) | 12.5x10⁻⁶ (12.5) |
| 40 | 12.5x10⁻⁶ (12.5) | 16.3x10⁻⁶ (16.3) |
| 50 | 16.3x10⁻⁶ (16.3) | 21.9x10⁻⁶ (21.9) |
| 60 | 21.9x10⁻⁶ (21.9) | 26.1x10⁻⁶ (26.1) |
2) Multigrade oil shall meet the viscosity requirements and the Low Temperature Viscosity Cold Crank Simulation requirements of SAE Test Method J300 for the designated grade.
3) Viscosity Index, minimum per ASTM D 2270: 100 for SAE grades 30, 40 and Multigrade; 95 for SAE grades 50 and 60.
4) Flash Point, °C, minimum per ASTM D 92: 220 for SAE grades 30 and Multigrade; 225 for SAE grade 40; and 243 for SAE grades 50 and 60.
5) Pour Point, °C, maximum per ASTM D 97: -24 for SAE grade 30; -22 for SAE grade 40; and -18 for SAE grades 50 and 60.
6) Viscosity, High Temperature, High Shear at 150°C, Pas (cP), minimum per ASTM D 4683, D 4741, D 4624: 3,3x10⁻³ Pas (3.3) for all viscosity grades.
7) Total Acid Number, mg KOH/g, maximum (titrated to a pH 11 end point) per ASTM D 664: 1.0 for all viscosity grades.
8) Ash Content, Mass %, maximum per ASTM D 482: 0.006 for all viscosity grades.
9) Trace Sediment, mL/100 mL Oil, maximum per ASTM D 2273: 0.005 for all viscosity grades.
10) Copper Strip Corrosion, maximum rating per ASTM D 130: 1 after 3 hours @ 100°C for all viscosity grades; and 3 after 3 hours @ 204°C for all viscosity grades.
11) Foaming Tendency/Stability per ASTM D 892: Aerated Volume, mL, maximum for all viscosity grades per Sequences I, II and III: 50; Volume after 10 minutes, mL, maximum for all viscosity grades per Sequences 1, II, and III: 0.
12) Compatibility with other oils per FTM 791 Method 3403: All viscosity grades shall pass.
13) Elastomer Compatibility, % swelling, acceptable range for all viscosity grades after 72 hours per FTM 791 Method 3604 (except conducted with the specific materials and temperatures herein listed):
| Material | Test Temperature | Acceptable Limits |
|---|---|---|
| AMS-3217/1 | 70°C (158°F) | - 5 to + 5 |
| AMS-3217/4 | 150°C (302°F) | - 5 to + 5 |
| AMS-3217/5 | 150°C (302°F) | - 5 to + 5 |
| US Navy Silicone Rubber | 121°C (250°F) | 0 to + 20 |
14) Trace Metal Content, ppm, maximum for all viscosity grades, per test method of Paragraph 4.5.2 of MIL-L-22851D (1 December 1990) or equivalent: Iron, 5; Silver, 3; Aluminum, 7; Chromium, 5; Copper, 3; Magnesium, 3; Nickel, 3; Lead, 5; Silicon, 25; Tin, 10; Titanium, 2; Molybdenum, 4.

## Patentansprüche

1. Bleifreie Flugbenzinzusammensetzung, welche umfaßt
ein Gemisch von Kohlenwasserstoffen und mindestens eine darin gelöste Cyclopentadienylmangantricarbonylverbindung in einer Menge, daß die Benzinzusammensetzung einen minimalen Klopfwert entsprechend einer Oktanzahl von 100, gemessen nach ASTM-Testverfahren D2700, aufweist und wobei Motormethoden-Oktanbewertungen zu Flugtechnikbewertungen in einer in der ASTM-Spezifikation D910-90 beschriebenen Weise umgewandelt werden und wobei die Zusammensetzung weiter dadurch gekennzeichnet ist, daß sie aufweist:
a) eine Destillationstemperatur, bestimmt gemäß ASTM-Testverfahren D86, von 75°C (167°F) maximale Temperatur bei 10 % verdampft, von 75°C (167°F) maximale Temperatur bei 40 % verdampft, von 135°C (275°F) maximale Temperatur bei 90 % verdampft und einen Endsiedepunkt von 170°C (338°F) maximale Temperatur, wobei die Summe der Temperaturen bei 10 % und 50 % verdampft mindestens 152,8°C (307°F) beträgt, wobei die Gewinnung durch Destillation mindestens 97 % beträgt, wobei der Destillationsrückstand maximal 1,5 % und der Destillationsverlust maximal 1,5 % beträgt,
b) eine Verbrennungswärme, bestimmt nach ASTM-Testverfahren D1405 und errechnet aus Tabelle 1 davon von mindestens 4.354 x 10⁷ J/kg (18.720 btu/Pfund), oder eine Verbrennungswärme, bestimmt nach ASTM Testverfahren D2382, von mindestens 4.350 x 10⁷ J/kg (18.700 btu/Pfund), wobei das letztgenannte Verfahren bei einem Unterschied der beiden als Kontrolle dient,
c) einen Dampfdruck, bestimmt nach ASTM-Testverfahren D323 oder D2551, von mindestens 3.866,89 kg/m² (5,5 Psi) und maximal 4.921,49 kg/m² (7,0 Psi),
d) eine Kupferstreifenkorrosion, bestimmt nach ASTM-Testverfahren D130, von maximal 1,
e) einen potentiellen Schmierölrückstand (5-Stunden-Alterungs Schmierölrückstand), bestimmt nach ASTM-Testverfahren D873 von maximal 6 mg/100 ml oder einen potentiellen Schmierölrückstand (16-Stunden-Alterungs Schmierölrückstand_{,} bestimmt nach ASTM-Testverfahren D873), von 10 mg/100 ml,
f) einen Schwefelgehalt, bestimmt nach ASTM-Testverfahren D1266 oder D2622, von maximal 0,05 Gew.-%,
g) einen Gefrierpunkt, bestimmt nach ASTM-Testverfahren D2386, von maximal -57,8°C (-72°F), und
h) eine Wasserreaktion, bestimmt nach ASTM-Testverfahren D1094, wobei die eventuelle Volumenänderung ± 2ml nicht übersteigt.

2. Zusammensetzung nach Anspruch 1, wobei die Benzinzusammensetzung einen minimalen Klopfwert entsprechend einer Oktanzahl von 100 aufweist, bestimmt nach ASTM-Testverfahren D2700, und eine minimale Leistungszahl, auf-/abgerundet auf die nächste ganze Zahl, bestimmt nach ASTM-Testverfahren D909, von 130 aufweist.

3. Zusammensetzung nach Anspruch 1, wobei die Cyclopentadienylmangantricarbonylverbindung im wesentlichen aus Methylcyclopentadienylmangantricarbonyl besteht.

4. Verfahren zum Betrieb eines Viertakt-Hubkolbenflugzeugmotors, welches umfaßt
als Motorkraftstoff eine bleifreie Flugbenzinzusammensetzung zur Verfügung zu stellen oder zu verwenden, welche umfaßt
ein Gemisch von Kohlenwasserstoffen und mindestens eine darin gelöste Cyclopentadienylmangantricarbonylverbindung in einer Menge, daß die Benzinzusammensetzung einen minimalen Klopfwert entsprechend einer Oktanzahl von 100, gemessen nach ASTM-Testverfahren D2700, aufweist und wobei Motormethoden-Oktanbewertungen zu Flugtechnikbewertungen in einer in der ASTM-Spezifikation D910-90 beschriebenen Weise umgewandelt werden und wobei die Zusammensetzung weiter dadurch gekennzeichnet ist, daß sie aufweist
a) eine Destillationstemperatur, bestimmt gemäß ASTM-Testverfahren D86, von 75°C (167°F) maximale Temperatur bei 10 % verdampft, von 75°C (167°F) maximale Temperatur bei 40 % verdampft, von 135°C (275°F) maximale Temperatur bei 90 % verdampft und einen Endsiedepunkt von 170°C (338°F) maximale Temperatur, wobei die Summe der Temperaturen bei 10 % und 50 % verdampft mindestens 152,8°C (307°F) beträgt, wobei die Gewinnung durch Destillation mindestens 97 % beträgt, wobei der Destillationsrückstand maximal 1,5 % und der Destillationsverlust maximal 1,5 % beträgt,
b) eine Verbrennungswärme, bestimmt nach ASTM-Testverfahren D1405 und errechnet aus Tabelle 1 davon, von mindestens 4.354 x 10⁷ J/kg (18.720 btu/Pfund), oder eine Verbrennungswärme, bestimmt nach ASTM Testverfahren D2382, von mindestens 4.350 x 10⁷ J/kg (18.700 btu/Pfund) beträgt, wobei das letztgenannte Verfahren bei einem Unterschied der beiden als Kontrolle dient,
c) einen Dampfdruck, bestimmt nach ASTM-Testverfahren D323 oder D2551, von mindestens 3.866,89 kg/m² (5,5 Psi) und maximal 4.921,49 kg/m² (7,0 Psi) beträgt,
d) eine Kupferstreifenkorrosion, bestimmt nach ASTM-Testverfahren D130, von maximal 1,
e) einen potentiellen Schmierölrückstand (5-Stunden-Alterungs Schmierölrückstand), bestimmt nach ASTM-Testverfahren D873 von maximal 6 mg/100 ml oder einen potentiellen Schmierölrückstand (16-Stunden-Alterungs Schmierölrückstand, bestimmt nach ASTM-Testverfahren D873), von 10 mg/100 ml,
f) einen Schwefelgehalt, bestimmt nach ASTM-Testverfahren D1266 oder D 2622, von maximal 0,05 Gew.-%,
g) einen Gefrierpunkt, bestimmt nach ASTM-Testverfahren D2386, von maximal -57,8°C (-72°F), und
h) eine Wasserreaktion, bestimmt nach ASTM-Testverfahren D1094, wobei die eventuelle Volumenänderung ± 2ml nicht übersteigt.

5. Verfahren nach Anspruch 4, wobei die Benzinzusammensetzung einen minimalen Klopfwert entsprechend einer Oktanzahl von 100 aufweist, bestimmt nach ASTM-Testverfahren D2700, und eine minimale Leistungszahl, auf-/abgerundet auf die nächste ganze Zahl, bestimmt nach ASTM-Testverfahren D909, von 130 aufweist.

6. Verfahren nach Anspruch 4, wobei die Cyclopentadienylmangantricarbonylverbindung im wesentlichen aus Methylcyclopentadienylmangantricarbonyl besteht.

7. Verfahren zum Betrieb eines Viertakt-Hubkolbenflugzeugmotors nach Anspruch 4, welches zusätzlich umfaßt
als Schmieröl für den Motor eine Schmierölzusammensetzung zur Verfügung zu stellen oder zu verwenden, die den folgenden chemischen und physikalischen Eigenschaftsvoraussetzungen genügt:
1) Viskosität m²/s (cSt) nach ASTM D445:
| SAE-Gütegrad | Minimum bei 100°C | weniger als 100°C |
|---|---|---|
| 30 | 9,3 x 10⁻⁶ (9,3) | 12, 5 x 10⁻⁶ (12,5) |
| 40 | 12,5 x 10⁻⁶ (12,5) | 16,3 x 10⁻⁶ (16,3) |
| 50 | 16,3 x 10⁻⁶ (16,3) | 21,9 x 10⁻⁶ (21,9) |
| 60 | 21,9 x 10⁻⁶ (21,9) | 26,1 x 10⁻⁶ (26,1) |
2) Mehrbereichsöl soll den Viskositätserfordernisssen und der Viskositätskältestartsimulationserfordernissen bei tiefen Temperaturen des SAE-Testverfahrens J300 für den entsprechenden Gütegrad genügen.
3) Minimaler Viskositätsindex gemäß ASTM D2270: 100 für SAE-Gütegütegrade 30, 40 und Mehrbereich, 95 für SAE-Gütegrade 50 und 60.
4) Minimaler Flammpunkt, °C, gemäß ASTM D92: 220 für SAE-Gütegrade 30 und Mehrbereich, 225 für SAE-Gütegrad 40 und 243 für SAE-Gütegrade 50 und 60.
5) Maximaler Fließpunkt, °C, gemäß ASTM D97: -24 für SAE-Gütegrad 30, -22 für SAE-Gütegrad 40 und -18 für SAE-Gütegrade 50 und 60.
6) Minimale Hochtemperaturviskosität, Hochscherung bei 150°C, Pa (cP), gemäß ASTM D4683, D4741, D4624: 3,3 x 10⁻³ Pa (3,3) für alle Viskositätsgütegrade.
7) Maximale Gesamtsäurezahl, mg KOH/g (titriert bis zu einem Endpunkt von pH 11) gemäß ASTM D664: 1,0 für alle Viskositätsgütegrade.
8) Maximaler Aschegehalt, Massen-%, gemäß ASTM D482: 0,006 für alle Viskositätsgütegrade.
9) Maximales Spurensediment, ml/100 ml Öl, gemäß ASTM D2273: 0,005 für alle Viskositätsgütegrade.
10) Maximale Kupfersteifenkorrosion, Bewertung gemäß ASTM D130: 1 nach 3 Stunden @ 100°C für alle Viskositätsgütegrade, und 3 nach 3 Stunden @ 204°C für alle Viskositätsgütegrade.
11) Schäumungsneigung/Stabilität gemäß ASTM D892: belüftetes Volumen, ml, maximal für alle Viskositätsgütegrade für Sequenzen I, II und III: 50; Volumen nach 10 Minuten, ml, maximal für alle Viskositätsgütegrade für Sequenzen I, II und III: 0.
12) Verträglichkeit mit anderen Ölen gemäß FTM791 Verfahren 3403: alle Viskositätsgütegrade sollen genügen.
13) Elastomerverträglichkeit, % Anschwellen, verträglicher Bereich für alle Viskositätsgütegrade nach 72 Stunden gemäß FTM791 Verfahren 3604 (außer wenn mit den spezifischen, hier aufgeführten Materialien und Temperaturen durchgeführt):
| Material | Testtemperatur | Annehmbare Grenzen |
|---|---|---|
| AMS-3217/1 | 70°C (158°F) | -5 bis +5 |
| AMS-3217/4 | 150°C (302°F) | -5 bis +5 |
| AMS-3217/5 | 150°C (302°F) | -5 bis +5 |
| US-Navy Silikongummi | 121°C (250°F) | 0 bis +20 |
14) Maximaler Gehalt an Spurenmaterialien, ppm, für alle Viskositätsgütegrade, gemäß Testverfahren MIL-L-22851D Paragraph 4.5.2 (1. Dezember 1990) oder äquivalent: Eisen, 5; Silber, 3; Aluminium, 7; Chrom, 5; Kupfer, 3; Magnesium, 3; Nickel, 3; Blei, 5; Silikon, 25; Zinn, 10; Titan, 2; Molybdän, 4.

## Revendications

1. Composition d'essence sans plomb pour l'aviation, qui comprend un mélange d'hydrocarbures et d'au moins un composé de cyclopentadiényl-manganèse-tricarbonyle qui y est dissous en une quantité telle que cette composition d'essence ait un indice d'octane en régime pauvre, avec un taux minimal de cognement, égal à 100 comme déterminé par la méthode d'essai ASTM D2700 et dans laquelle les indices d'octane déterminés par la Méthode Moteur sont convertis en indices aviation de la manière décrite dans la norme ASTM D910-90, cette composition étant en outre caractérisée en ce qu'elle a :
a) une température de distillation telle que déterminée par la méthode d'essai ASTM D86, de 10 % évaporés à une température maximale de 75°C (167°F) ; 40 % évaporés à une température maximale de 75°C (167°F) ; 90 % évaporés à une température maximale de 135°C (275°F) ; et un point d'ébullition final à une température maximale de 170°C (338°F) ; la somme des températures correspondant à 10 et 50 % évaporés étant au minimum de 152,8°C (307°F) ; le pourcentage recueilli par distillation étant au minimum de 97 % ; le résidu de distillation étant au maximum de 1,5 % ; et la perte à la distillation étant au maximum de 1,5 % ;
b) une chaleur de combustion, déterminée par la méthode d'essai ASTM D1405 et telle que calculée d'après son Tableau 1, de 4,354x10⁷ J/kg (18 720 btu par lb) au minimum, ou une chaleur de combustion telle que déterminée par la méthode d'essai ASTM D2382 de 4,350x10⁷ J/kg (18 700 btu par lb) au minimum, cette dernière méthode prévalant en cas de différence entre les deux ;
c) une pression de vapeur, telle que déterminée par la méthode d'essai ASTM D323 ou D2551, de 3866,89 kg/m² (5,5 lb/in²) au minimum et de 4921,49 kg/m² (7,0 lb/in²) au maximum ;
d) une corrosion d'une lame de cuivre, telle que déterminée par la méthode d'essai ASTM D130, numéro 1 au maximum ;
e) une gomme potentielle (gomme après 5 heures de vieillissement) telle que déterminée par la méthode d'essai ASTM D873, de 6 mg par 100 ml au maximum, ou une gomme potentielle (gomme après vieillissement pendant 16 heures comme déterminé par la méthode d'essai ASTM D873) de 10 mg par 100 ml ;
f) une teneur en soufre, telle que déterminée par la méthode d'essai ASTM D1266 ou D2622, de 0,05 % en poids au maximum ;
g) un point de congélation, tel que déterminé par la méthode d'essai ASTM D2386, de -57,8°C (-72°F) au maximum ; et
h) une réaction avec l'eau, telle que déterminée par la méthode d'essai ASTM D1094, dans laquelle la variation éventuelle de volume n'excède pas ± 2ml.

2. Composition suivant la revendication 1, dans laquelle la composition d'essence en question a un indice d'octane en régime pauvre avec un taux minimal de cognement égal à 100, tel que déterminé par la méthode d'essai ASTM D2700, et un coefficient minimal d'efficacité, rapporté au nombre entier le plus proche et tel que déterminé par la méthode d'essai ASTM D909, égal à 130.

3. Composition suivant la revendication 1, dans laquelle le composé de cyclopentadiényl-manganèse-tricarbonyle consiste essentiellement en méthylcyclopentadiényl-manganèse-tricarbonyle.

4. Procédé pour faire fonctionner un moteur d'aviation à quatre temps à pistons alternatifs, qui consiste A) à prévoir ou à utiliser comme carburant pour ce moteur une composition d'essence sans plomb pour l'aviation qui comprend un mélange d'hydrocarbures et d'au moins un composé de cyclopentadiényl-manganèse-tricarbonyle qui y est dissous en une quantité telle que cette composition d'essence ait un indice d'octane en régime pauvre, avec un taux minimal de cognement, égal à 100 comme déterminé par la méthode d'essai ASTM D2700 et dans laquelle les indices d'octane déterminés par la Méthode Moteur sont convertis en indices aviation de la manière décrite dans la norme ASTM D910-90, cette composition étant en outre caractérisée en ce qu'elle a :
a) une température de distillation telle que déterminée par la méthode d'essai ASTM D86, de 10 % évaporés à une température maximale de 75°C (167°F) ; 40 % évaporés à une température maximale de 75°C (167°F) ; 90 % évaporés à une température maximale de 135°C (275°F) ; et un point d'ébullition final à une température maximale de 170°C (338°F) ; la somme des températures correspondant à 10 et 50 % évaporés étant au minium de 152,8°C (307°F) ; le pourcentage recueilli par distillation étant au minimum de 97 % ; le résidu de distillation étant au maximum de 1,5 % ; et la perte à la distillation étant au maximum de 1,5 % ;
b) une chaleur de combustion, déterminée par la méthode d'essai ASTM D1405 et telle que calculée d'après son Tableau 1, de 4,354x10⁷ J/kg (18 720 btu par lb) au minimum, ou une chaleur de combustion telle que déterminée par la méthode d'essai ASTM D2382 de 4,350x10⁷ J/kg (18 700 btu par lb) au minimum, cette dernière méthode prévalant en cas de différence entre les deux ;
c) une pression de vapeur, telle que déterminée par la méthode d'essai ASTM D323 ou D2551, de 3866,89 kg/m² (5,5 lb/in²) au minimum et de 4921,49 kg/m² (7,0 lb/in²) au maximum ;
d) une corrosion d'une lame de cuivre, telle que déterminée par la méthode d'essai ASTM D130, numéro 1 au maximum ;
e) une gomme potentielle (gomme après 5 heures de vieillissement) telle que déterminée par la méthode d'essai ASTM D873, de 6 mg par 100 ml au maximum, ou une gomme potentielle (gomme après vieillissement pendant 16 heures comme déterminé par la méthode d'essai ASTM D873) de 10 mg par 100 ml ;
f) une teneur en soufre, telle que déterminée par la méthode d'essai ASTM D1266 ou D2622, de 0,05 % en poids au maximum ;
g) un point de congélation, tel que déterminé par la méthode d'essai ASTM D2386, de -57,8°C (-72°F) au maximum ; et
h) une réaction avec l'eau, telle que déterminée par la méthode d'essai ASTM D1094, dans laquelle la variation éventuelle de volume n'excède pas ± 2ml.

5. Procédé suivant la revendication 4, dans lequel la composition d'essence a un indice d'octane en régime pauvre, avec un taux minimal de cognement, égal à 100 comme déterminé par la méthode d'essai ASTM D2700 et un coefficient minimal d'efficacité, rapporté au nombre entier le plus proche et comme déterminé par la méthode d'essai ASTM D909, égal à 130.

6. Procédé suivant la revendication 4, dans lequel le composé de cyclopentadiényl-manganèse-tricarbonyle consiste essentiellement en méthylcyclopentadiénylmanganèse-tricarbonyle.

7. Procédé pour faire fonctionner un moteur d'aviation à quatre cycles à pistons alternatifs suivant la revendication 4, qui consiste en outre à prévoir et/ou à utiliser comme huile lubrifiante pour ce moteur une composition d'huile lubrifiante qui satisfait aux conditions de propriétés chimiques et physiques suivantes :
1) viscosité en m²/s (cSt) d'après la norme ASTM D445 :
| Grade SAE | Minimum à 100°C | En dessous de 100°C |
|---|---|---|
| 30 | 9,3x10⁻⁶ (9,3) | 12,5x10⁻⁶ (12,5) |
| 40 | 12,5x10⁻⁶ (12,5) | 16,3x10⁻⁶ (16,3) |
| 50 | 16,3x10⁻⁶ (16,3) | 21,9x10⁻⁶ (21,9) |
| 60 | 21,9x10⁻⁶ (21,9) | 26,1x10⁻⁶ (26,1) |
2) Huile multigrade doit satisfaire aux conditions de viscosité et aux conditions de démarrage à froid à basse température de la méthode d'essai SAE J300 pour le grade désiré.
3) Indice de viscosité, minimum d'après la méthode ASTM D2270 : 100 pour les grades SAE 30, 40 et un Multigrade ; à 95 pour les grades SAE 50 et 60.
4) Point d'éclair, °C, minimum d'après la norme ASTM D92 : 220 pour grade 30 SAE et multigrade ; 225 pour grade SAE 40 ; et 243 pour les grades SAE 50 et 60.
5) Point d'écoulement, °C, maximum d'après la norme ASTM D97 : -24 pour le grade SAE 30 ; -22 pour le grade SAE 40 ; et -18 pour les grades SAE 50 et 60.
6) Viscosité à haute température et sous fort cisaillement à 150°C, en Pa.s (cP), minium d'après la norme ASTM D4683, D4741, D4624 : 3,3x10⁻³ Pa.s (3,3) pour tous les grades de viscosité.
7) Indice d'aciditité totale, en mg de KOH/g, maximum (titré jusqu'à un point de virage à pH 11) d'après la norme ASTM D664 : 1,0 pour tous les grades de viscosité.
8) Teneur en cendres, en % en masse, maximum d'après la norme ASTM D482 : 0,006 pour tous les grades de viscosité.
9) Sédiment à l'état de traces, ml/100 ml d'huile, maximum d'après la norme ASTM D2273 : 0,005 pour tous les grades de viscosité.
10) Corrosion d'une lame de cuivre, indice maximal d'après la norme ASTM D130 : 1 après 3 heures à 100°C pour tous les grades de viscosité ; et 3 après 3 heures à 204°C pour tous les grades de viscosité.
11) Tendance/stabilité au moussage d'après la norme ASTM D892 : volume aéré, ml, maximum pour tous les grades de viscosité d'après les Séquences I, II et III : 50 ; volume après 10 minutes, ml, maximum pour tous les grades de viscosité d'après les Séquences I, II et III : 0.
12) Compatibilité avec d'autres huiles d'après FTM 791, méthode 3403 : tous les grades de viscosité doivent être admis.
13) Compatibilité avec les élastomères, % de gonflement, plage admissible pour tous les grades de viscosité après 72 heures d'après FTM 791, méthode 3604 (excepté la conduite avec les matériaux particuliers et aux températures énumérées ici) :
| Matériau | Température d'essai | Limites admissibles |
|---|---|---|
| AMS-3217/1 | 70°C (158°F) | - 5 à + 5 |
| AMS-3217/4 | 150°C (302°F) | - 5 à + 5 |
| AMS-3217/5 | 150°C (302°F) | - 5 à + 5 |
| Caoutchouc siliconé US Navy | 121°C (250°F) | 0 à + 20 |
14) Teneur en métaux à l'état de traces, ppm, maximums pour tous les grades de viscosité, d'après la méthode d'essai du paragraphe 4.5.2 de la norme MIL-L-22851D (1 Décembre 1990) ou l'équivalent : fer, 5 ; argent, 3 ; aluminium, 7 ; chrome, 5 ; cuivre, 3 ; magnésium, 3 ; nickel, 3 ; plomb, 5 ; silicium, 25 ; étain, 10 ; titane, 2 ; molybdène, 4.
